

## UNITED STATES PATENT OFFICE

GLENN W. TRAER, OF CHICAGO, ILLINOIS, ASSIGNOR TO NORTHERN LIGNITE COAL COMPANY, OF CHICAGO, ILLINOIS, A CORPORATION OF DELAWARE

## PROCESS OF PRODUCING AN ARTIFICIAL FUEL

No Drawing.

Application filed June 15, 1925. Serial No. 37,384.

This invention relates to improvements in artificial fuel and process of producing the same.

This invention more particularly relates to an artificial fuel and the process of producing the same from coking coal whose coking properties have been removed. The fuel produced is in the nature of what is well known in the art as "char", which is a much more desirable fuel for general purposes, and especially in briquettes for domestic use, than high volatile coking coals.

It is common practice to reduce caking or coking coals to coke by depriving the coking coal of its volatile constituents by heating it in a retort or oven to a degree above its melting or fusion point, so that the resultant coke is in a practically common mass and is mainly fixed carbon in a substantially homocellular or porous state. But this novel fuel is not coke and such coking is prevented.

The parts of coking coal which cause coking in ordinary processes are believed to be bituminous and resinous matters which, when heated to a sufficient degree, partly will volatilize and partly will melt; those which volatilize will pass off and those which do not volatilize, unite with the fixed carbon to form the hard cellular mass known as coke. Some of these hydrocarbons will volatilize at lower temperatures than are required to melt and fuse the coal into a mass. It is the custom in coking practice to subject the body of coal to the highest degree of heat required for coking as early in the process of heating as is practicable and to maintain the heat at such degree throughout the process. It has been observed that volatilization begins at or about six hundred degrees Fahrenheit (600°), and that melting or fusion begins at or about seven hundred degrees Fahrenheit (700°). These temperatures have variations for different coals; incipient volatilization appears to begin between 550° F. and 600° F. in various coals and incipient fusion appears to begin at temperatures varying from perhaps 680° F. to perhaps 720° F.

I have discovered that the coking property is eliminated from coking coal if the portion of the bituminous matter which will volati-

lize at degrees of heat below the melting or fusion point is driven off; and that melting or fusion will not take place and mass coke will not be formed from coking coal which has been so treated, even though the coal be then subjected to a sufficient degree of heat to drive off all recondensable matters. This process requires that in this second stage the coal be heated to a temperature of approximately 800° to 1100° F.

A large part of the bituminous matter which is volatilized in the coking process is recondensable into tar and the remainder passes off as fixed gas. That part which is recondensable is the cause of smoke when bituminous coal is burned in many of the common practical methods of combustion. In ordinary methods of combustion, bituminous coking coal to a considerable degree melts in the firebox, tending to blanket the grate, resulting in obstructions to the circulation of air through the body of fuel and interfering with efficient combustion.

Coking coal which has been passed through the first stage only of this new and novel process, has had all moisture eliminated from it, thereby largely increasing its fuel value, and when burned in common practical methods will not melt in the firebox; proper circulation of air through the body of fuel is thereby facilitated, smoke is lessened and combustion is made more efficient. When the coal, which also has been passed through the second stage of this process, is burned in common practical methods, the formation of smoke is entirely eliminated and efficient combustion still further promoted.

The object therefore of this invention is to provide an artificial dry, partially volatile and smokeless, fuel and process of producing the same.

Other objects of the invention will more fully appear from the following description and will be pointed out in the annexed claims.

In producing this artificial fuel there may be employed any of the common forms of ovens or retorts which may be recognized as suitable for the purpose.

The size of the coking coal used is not more than two inches. Internal heat is ap-

plied by passing gases through the mass, while the same is maintained in a loose state and is thus directly heated.

The caking or coking coal from which the fuel is to be made is placed within the oven or retort and heated, to certain ranges of heat under control so that, after it has been so treated, it can thereafter, be subjected to higher ranges of heat which would have caused coking except for such prior heat-treatment. In other words, this treatment prevents the coking of coking coals. The fuel which has been so treated is preserved in substantially the same form as it was prior to such treatment. After such novel treatment of coking coal, the resultant fuel may be heated in the oven or retort up beyond the coal's former fusion point and it will not coke while further smoky and tarry volatiles are driven off so as to produce a substantially non-smoking, non-coking fuel. If desired, such fuel may be ground and briquetted by the addition of pitch and a small percentage of coking coal and/or glutinous matter.

In producing this novel fuel and carrying out this process, a coking coal so placed in a suitable retort or oven is heated to its incipient volatilization temperature. This should be at least six hundred degrees (600°) F. as it has been observed that substantially no volatilization is produced by a lower temperature upon the various coking coals used. The upper permissible limit of temperature is the fusion point of the coal and it varies somewhat with the particular coking coals used but so far as applicant is now aware, such upper limit should not exceed substantially seven hundred degrees (700°) F. The volatilization of the coking coal so heated, between these volatilization and fusion points, may be observed by the emission of smoke and vapors.

The period of time during which the coking coal is maintained between the permissible limits varies with the composition of the different coking coals from different mines but in actual practice is sufficient to raise the temperature of the coal being treated until the characteristic smoke or vapor is being driven off, care being taken not to permit the temperature of the treated coal to exceed the fusion point, at least until after the cessation of emission of the smoke or vapor while the coal is being maintained at a temperature below the fusion point.

After this new fuel is obtained, it may then be utilized as such; or, it may then be further distilled in the retort to drive off further volatiles as above described; and useful gases and tar thereby recovered and the residual fuel substantially in the form of a char be employed as a fuel. Likewise, this char may thereafter be briquetted. One form of such briquetting is above suggested as by crushing the fuel and then adding pitch and a relative-

ly small percentage of coking coal and/or glutinous matter and then forming into small blocks or briquettes by pressure.

Having thus described my invention, what I claim as new and desire to secure by Letters Patent, is:

1. A process of producing a non-coking fuel from a coking coal which comprises in subjecting the coking coal to a temperature above its incipient volatilization temperature and below its fusion temperature and maintaining the temperature of the coal between these temperatures until emission of volatiles characteristic of that temperature range substantially ceases. 80

2. A process of producing a non-coking fuel from a coking coal which comprises subjecting the coking coal to a temperature above its incipient volatilization temperature and below its fusion temperature and maintaining the coal-temperature between these temperatures until the coking tendency has been practically eliminated. 85

3. A process of producing a non-coking and smokeless fuel from a coking coal which comprises subjecting the coking coal to a temperature above its incipient volatilization temperature and below its fusion temperature and maintaining the coal-temperature between these temperatures until the coking 95 tendency has been practically eliminated; and then subjecting the coal to a higher degree of heat sufficient so as to drive off substantially all the tarry and smoky volatile substances without causing the coal to substantially change its form. 100

4. A process of producing a non-coking fuel from a coking coal which comprises subjecting the coal to temperatures substantially within the range of from 600 degrees Fahrenheit to 700 degrees Fahrenheit, and maintaining the coal within this range until emission of volatiles substantially ceases. 105

5. A process of producing a non-coking fuel from a coking coal which comprises subjecting the coal to temperatures not less than 600 degrees Fahrenheit and not more than 700 degrees Fahrenheit and maintaining the charge within this range until emission of volatiles substantially ceases. 110

In witness whereof, I have hereunto set my hand this 12 day of June 1925.

GLENN W. TRAER.

120

125

130